

## UNITED STATES PATENT OFFICE.

ALADAR PACZ, OF CLEVELAND HEIGHTS, OHIO, ASSIGNOR TO GENERAL ELECTRIC COMPANY, A CORPORATION OF NEW YORK.

## PROCESS OF PREPARING BORON-IRON ALLOYS.

No Drawing. Application filed May 3, 1919, Serial No. 294,456. Renewed April 7, 1925.

To all whom it may concern:

Be it known that I, ALADAR PACZ, a citizen of the United States, residing at Cleveland Heights, in the county of Cuyahoga, 5 State of Ohio, have invented certain new and useful Improvements in Processes of Preparing Boron-Iron Alloys, of which the following is a specification.

My invention relates to so-called alloy 10 steels and to methods and means for rendering them more easily fusible and therefore rendering them of more service in the arts. These steels include one or more of the rarer metals such as tungsten, chromium, 15 vanadian, manganese, silicon, nickel, molybdenum, zirconium, tantalum, uranium, columbium, cobalt and others. The use of my invention makes it feasible to cast such steels into articles which have heretofore 20 been made by forging or otherwise working the metal. It also improves the quality of such alloy steels as are ultimately forged or otherwise worked.

According to my invention, boron is 25 incorporated in the steel along with one or more of the aforesaid rarer metals. The action of the boron is probably to alloy with the steel as well as to act as a scavenger. This is to be distinguished from the 30 action of such materials as boric acid and other boron compounds.

The amount of boron in the final product may vary depending upon the degree of fusibility desired. The best results are 35 obtained when from three-fourths per cent to four or five per cent boron are included in the final steel and, when a greater amount is included, the results are not so satisfactory both from the standpoint of economy and 40 effect obtained. The amount of boron will depend to a certain extent on the carbon content since the higher carbon steels have generally the lower melting points.

One application of my invention is to the 45 production of high speed steel which can be cast readily into cutters and other tools. In one instance, a high speed steel containing three-fourths per cent boron, seventeen per cent tungsten, five per cent chromium, three- 50 fourths per cent vanadium and sixty-five one-hundredths per cent carbon was cast into a cutting tool. Hammer dies were made from a steel containing three-tenths per cent vanadium, one and one-half per 55 cent chromium, and four-tenths per cent

boron. Examples of the many alloy steels to which my invention is applicable are the so-called stainless steels, motor valve steels and construction steels, for instance those used for automobile parts and machinery in 60 general. By incorporating a relatively small per cent of the boron with the other alloy metals such as the tungsten and others hereinbefore referred to, a comparatively easily fusible steel is obtained which can be 65 cast readily even into intricate forms substantially free from blow holes and other defects and which still preserves the properties which are given to the metal by the alloying element exclusive of the boron. 70

I have produced steels with a low content of nickel or chromium, for instance one and four-tenths per cent nickel or one and two-tenths per cent chromium, with one-tenth to two-tenths per cent boron which had 75 physical characteristics equal or superior to those of steels having much higher contents of the nickel or chromium but containing no boron. It is true that when such small proportions of boron are incorporated the 80 effect on the melting point is not so pronounced and by incorporating more boron the fusibility may be increased. From this standpoint my invention comprises the utilization of boron to replace a part of the 85 other rarer metals such as nickel, chromium and others.

I prefer to introduce the boron alloyed with other metals, usually iron. It is desirable also to have a certain amount of 90 aluminum or aluminum and silicon present. This result is obtained preferably by utilizing the alumino-thermic method for the production of the boron alloy. This method consists in mixing together the oxides of 95 the alloying metals including a certain amount of boron compound such as boric acid and aluminum and igniting the mixture. I prefer to utilize the alumino-thermic method which is disclosed in my co-pending application Serial No. 255,790 filed September 26, 1918, in which specific reference is made to a method of producing an alloy of zirconium. According to that method, the materials are made into briquettes consisting of the oxides of the various alloying metals and finely divided aluminum preferably of the blown variety. A certain amount of flaky aluminum can be incorporated in the briquettes, at least in the 110

briquette which is initially ignited, since this method contemplates the ignition of one or more briquettes initially and the addition subsequently, of enough briquettes to produce the desired amount of alloy. The oxides of the tungsten, chromium or other metal to be incorporated in the alloy may be included in the briquette so that the metal will be reduced at the same time as the boron. It is a fact that the presence of the boron improves the alloy because its effect in lowering the melting causes the alloy to be more readily absorbed when added to metal baths. To produce an alloy containing approximately sixteen per cent boron, a mixture of one thousand and fifty grams of  $Fe_3O_4$ , six hundred and thirty grams of  $B_2O_3$ , seven hundred and seventy grams of finely divided aluminum of the blown variety and fifteen grams of the flaky aluminum were mixed and formed into a briquette with the addition of sodium silicate as a binder. The reaction was started preferably by igniting a small briquette having a high per cent of the flaky aluminum in a blast lamp and dropping it into a crucible containing a number of briquettes of the composition just described. After the reaction has progressed, more briquettes were added until the desired amount of product was obtained. This product contained about three to six per cent aluminum and a slight amount of silicon derived from the binder. As hereinbefore stated, the aluminum and silicon are of advantage since they have a very efficient deoxidizing action.

The boron alloy produced as above described may be added to the molten bath of the other metals or otherwise incorporated. Preferably the materials added to the molten bath contains not only the boron but also the other rare metal or metals.

Most of the specific steels hereinbefore referred to will be found to contain in addition to the boron and iron at least one other

metal of the iron or chromium groups and it is with such steels that my best results have been secured.

What I claim as new and desire to secure by Letters Patent of the United States, is:—

1. The process of making an alloy containing boron which consists in briquetting a boron compound with a compound of another metal and finely divided aluminum, and igniting the briquette to cause the said materials to react.

2. The process of making an alloy containing iron and boron which consists in briquetting a boron compound with an iron compound and finely divided aluminum, and igniting the briquette to cause a reaction between the said materials.

3. The process of making an alloy containing iron, boron and another metal which consists in briquetting a boron compound, an iron compound and a compound of the other metal with finely divided aluminum, and igniting the briquette to cause a reaction between the said materials.

4. The process of making an alloy containing iron and boron which consists in briquetting oxides of boron and iron with finely divided aluminum, and igniting the briquette to cause a reaction between the said materials.

5. The process of producing an alloy containing iron and boron which consists in briquetting oxides of boron and iron with finely divided aluminum of the blown variety, and igniting the briquette to cause a reaction between the said materials.

6. The process of producing ferro-boron which consists in briquetting oxides of boron and iron with finely divided aluminum, and igniting the briquette to produce a reaction between the said materials.

In witness whereof, I have hereunto set my hand this first day of May, 1919.

ALADAR PACZ.